

Patented Nov. 28, 1922.

## UNITED STATES PATENT OFFICE.

JERE SCANLAN, OF DEARBORN, AND HENRY GARDNER, OF DETROIT, MICHIGAN.

## RUSTPROOFING COATING.

No Drawing.

Application filed March 22, 1922. Serial No. 545,874.

*To all whom it may concern:*

Be it known that we, JERE SCANLAN and HENRY GARDNER, citizens of the United States, residing at 133 Mason Street north, 5 Dearborn, and 2745 Third Avenue, Detroit, respectively, in the county of Wayne and State of Michigan, have invented new and useful Improvements in a Rustproofing Coating, of which the following is a specification.

The object of our invention is to provide a rust-proofing for metals and a method for accomplishing the rust-proofing which is simple, and inexpensive while being, at the 15 same time, durable.

A further object of our invention is to provide a rust proof coating for metals, such as iron or steel, which will really prevent rust on the surface of such metals so long as 20 the coating remains intact and which at the same time will have a black or other color so that the metal may be finished over the rust proof coating with any suitable coloring of siccative material.

25 A further object of our invention is to utilize a known method of rust-proofing in combination with means for coloring such rust proof coating to conform to the color of the finish with which the metal is to be 30 coated.

With these and other objects in view, our invention consists in the process of forming the coating and the coating itself as described in this specification and set forth in 35 the claims.

In the practise of our invention we first coat the material to be rust proofed, such as iron or steel or any metal of a ferrous nature, with zinc or zinc alloy plating by any 40 of the well known methods for forming such platings such for instance as by electrolysis. The method of coating or plating the material with zinc will not be here more particularly described because it forms no part of 45 the invention in connection with this application.

In connection with zinc plating, we believe that this type of rust proof coating for ferrous metals is superior, in so far as preventing rust is concerned, to any other type of 50 rust preventative coating. Zinc plating, however, is subject to the disadvantage that it cannot be successfully enameled or lacquered for use in connection with metals 55 which are exposed to the weather and which require a high finish such for instance as au-

tomobile parts. Where such coatings of varnish or the like are attempted over zinc plating a large number of such coatings are required in order to give a pure black color to 60 the material and even then the coating tends to chip off when it becomes thoroughly dry. In fact the enameling of zinc plating, so far as we know, is conceded to be impracticable, 65 commercially.

After the material to be rust proofed has been so coated with the zinc we then subject it to a hot bath of an antimony solution which will form on the zinc a closely adhering metallic deposit of dead black or 70 other color which can be given a very beautiful finish by simply applying thereto one coat of enamel.

By our invention we are, therefore, enabled to secure the well known advantages of 75 the zinc plate rust proofing together with a decrease in the number of coats of enamel required to secure any desired finish on the metal, thereby securing a durable and desirable finish for steel parts or for ferrous parts 80 which are to be exposed to the weather and which require a high finish.

In the practice of our process we have experimented with various thicknesses of zinc plating with various solutions of antimony, 85 and with various times for exposure of the plated article to the antimony. We were very successful in accomplishing our coating of the zinc plated article with the metallic antimony by dipping articles into a very 90 hot solution of butter of antimony (antimony chloride diluted in the proportion of one part antimony chloride, British Pharmacopia strength, to 1200 parts water). Where one pint of the butter of antimony 95 was used to 150 gallons of water, the water was brought to a temperature averaging the boiling point. Caustic soda to the amount of two pounds was added to this solution.

Our experiments show, however, that it is 100 not necessary to use caustic soda, (NaOH) for an alkali in connection with this solution, as good success was obtained from potassium salts and more particularly from potassium carbonate, ( $K_2CO_3$ ), or from sodium hydroxide. Our experiments further show that other salts of antimony than antimony chloride  $SbCl_3$  and other salts which fall into the same class with antimony chloride, namely, 105 arsenic, bismuth, and phosphorus, may be 110 used.

In fact our invention consists in the col-

oring of the rust preventing zinc coating on various metals by means of some compound of the antimony group, an acid forming element such as chlorine and an alkaline solution.

The point of using the caustic soda or other alkali is to neutralize the disintegrating effect of the acid used with the antimony compound, as this acid tends to disintegrate 10 the zinc coating thereby lessening its rust proofing ability. Where, however, a slightly alkaline, neutral, or a very slightly acid solution of a salt of antimony is used, practically no disintegration of the zinc coating 15 takes place, and a very even deposit of metallic antimony may be formed on the zinc. The thickness of this deposit depends upon the relative proportion of antimony in the solution and the length of time that the article 20 is left in the solution. For instance, an article left in the solution made as described above, for approximately three minutes will have a very good coating of metallic antimony deposited thereon.

25 The advantages of our improved method of rust proofing are believed to have been brought out in the main in the specification hereinafter, but it should be again pointed out that by our process we are enabled to 30 secure the advantages of the best rust proof coating with which we are familiar and at the same time we are enabled to provide a ferrous article with a very high finish with but very few coats or one siccative coating.

35 It will be understood that some variations may be made in the proportions of the solution herein described and that the temperature may be varied somewhat, changes in the proportions resulting, however, in corresponding increases or decreases in the time 40 for a coating to be formed, and changes in the heat of the solution resulting similarly. Different salts of antimony will be used also to give colors other than black. These coatings, however, of other colors are not herein 45 more fully set forth as it is not our desire to cover by this application any particular method of coating ferrous material to obtain any color other than black as each such color 50 is obtained by varying the salt of antimony used, so that we desire to cover the methods of obtaining the specific colors separately, and to cover the method of producing the black, and the method generally, in this application.

What we claim is:

1. The method of coating the surfaces of ferrous articles for rust proofing consisting of first plating such surfaces with zinc or 60 zinc compounds and then depositing metallic antimony on the plated surfaces.

2. The method of coating the surfaces of ferrous articles for rust proofing consisting of first plating the articles with zinc or zinc compounds, then coating the plated surface 65 with metallic antimony, and coating the surface thus formed with a siccative coating.

3. The method of rust proofing ferrous surfaces consisting of first plating the surface with zinc or zinc compounds and then 70 subjecting the plated surface to the action of a solution of antimony chloride.

4. The method of rust proofing ferrous surfaces consisting of first plating such surfaces with zinc or zinc compounds and then 75 subjecting the plated surfaces to the action of a hot solution of a salt of antimony and a forming acid.

5. The method of rust proofing a ferrous surface consisting of first coating the surface 80 with zinc then subjecting it to a solution of a salt of antimony and a forming acid, and then coating the surface thus formed with a siccative coating.

6. The method of rust proofing ferrous 85 surfaces consisting of zinc plating such surfaces and then subjecting them to a hot bath formed from a solution of a salt of antimony, a forming acid, and an alkali.

7. The method of rust proofing ferrous 90 surface consisting of zinc plating the surface and then subjecting it to the action of a hot solution of a salt of antimony, an acid, and sufficient alkali to render the solution near neutral.

8. The method of rust proofing of ferrous surfaces consisting of zinc plating such surfaces and then subjecting the plated surfaces to a substantially neutralized acid solution of a salt of antimony. 95

9. The method of coating ferrous surfaces for rust proofing consisting of zinc plating the surfaces and then subjecting them to a hot bath formed from a solution of a salt of antimony, an acid, and potassium salts. 100

10. The method of rust proofing ferrous surfaces consisting of zinc plating the surfaces and then subjecting them to a solution of antimony chloride and caustic soda in substantially the proportions of one pint of 110 antimony chloride, two pounds of caustic soda, and one hundred and fifty gallons of water.

11. The method of rust proofing of ferrous surfaces consisting of zinc plating such surfaces and then subjecting the plated surfaces to a substantially neutralized acid solution of a salt of antimony substantially in the proportions specified. 115

February 6, 1922.

JERE SCANLAN.  
HENRY GARDNER.